

Nov. 27, 1928.

1,693,429

A. O. AUSTIN

## METHOD OF CASTING

Filed July 2, 1926



Patented Nov. 27, 1928.

1,693,429

# UNITED STATES PATENT OFFICE.

ARTHUR O. AUSTIN, OF BARBERTON, OHIO, ASSIGNOR, BY MESNE ASSIGNMENTS, TO THE OHIO BRASS COMPANY, OF MANSFIELD, OHIO, A CORPORATION OF NEW JERSEY.

## METHOD OF CASTING.

Application filed July 2, 1926. Serial No. 120,090.

This invention relates to the manufacture of ceramic ware and has for its object the provision of a method by which articles of this nature may be more quickly and efficiently manufactured by casting than has heretofore been possible and by which many articles may be cast that heretofore could not be made by this method.

The invention is exemplified in the steps in the process, described in the following specification and illustrated in the accompanying drawing.

In the drawing—

Fig. 1 is an elevation of half of a mould showing the formed piece and other parts in section.

Many ceramic articles may be formed by what is known as the casting method in which a mould of plaster of Paris or other porous material is filled with slip in which the clay is mixed with water and the water allowed to pass by capillary action through the wall of the mould leaving a layer of clay deposited on the inner surface of the mould.

In the formation of ceramic articles by the casting process it is often very difficult or impossible to form pieces with certain body compositions which will not crack during the casting process. The time required in casting as well as the corrosion of the plaster of Paris moulds used is also another serious objection to using the casting process in many operations. The dissolving or disintegration of the plaster of Paris moulds not only tends to reduce the useful life of the mould, but in many cases causes a change in the casting slip which makes casting exceedingly difficult.

In the ordinary casting process the mould has to be capable of absorbing water so that the cast piece will build up on the walls of the mould by hardening of the slip due to the absorption of water. In general, this limits the nature of the material which can be used for forming moulds to plaster of Paris. Since the plaster of Paris is not very strong, small pieces breaking off and getting into the casting slip or pieces of ware adjacent to the mould tend to spoil the properties of the slip so that the casting and burning properties in many cases are materially changed. The fouling of the casting slip from material absorbed from the moulds and entering the slip directly or through chips from the moulds, or by defective cast pieces which are returned to the slip, is a serious item and causes losses and

irregularities in the casting process. Another difficulty in casting is encountered owing to the fact that the portion of the cast piece next to the mould is dense while the surface in contact with the casting slip contains a much larger percentage of water. During the drying operation the portion containing the larger percentage of water tends to shrink more than the denser part which shrinkage is resisted by the portion adjacent the mould so that in many cases a check or crack develops owing to the stress set up.

The present method is designed to eliminate this difficulty to a very large extent and at the same time facilitate the casting operation.

Fig. 1 shows one half of a casting mould used in the process to which this invention refers, also a section through the piece of ware or the article being formed. In the ordinary casting process it is necessary to use slips in many cases which will shrink but little during the casting, as it is necessary to keep the cast material in contact with the mould so the capillary attraction will be maintained in order that the piece will be built up to the desired thickness. Many desirable casting slips can not be used to advantage owing to the fact that the time required in casting is so long that the piece begins to shrink forming air pockets or films between the surface of the cast article and the mould which destroy the capillary absorption of the mould. In the improved method this is practically eliminated or reduced so that it is not a serious factor and permits the use of casting slips which it would not be possible to use in the ordinary method.

In the form of the invention shown in Fig. 1 a steel or metal case 10 with holes 11 for clamping the two halves together is lined with a plaster or other porous lining 12. The inner surface 13 of the plaster conforms to the outline of the piece 14 which it is desired to form. The particular piece shown is a bushing, but it is evident that the method may be applied to practically any form of ceramic ware and is particularly adaptable to sanitary ware, electrical porcelain or other complicated shapes.

The entrance to the inside of the mould is obtained through pipe connections 15 and 16 which are usually provided with valves 17 and 18 connected to hose connections 19 and 20. The piece 14 has an undercut on the outer surface, hence it is necessary to use split

rings 21 and 22. While these rings are usually of the same composition as the mould, they may be made of metal, wax, or other material in many cases. The ring 21 is shown as made of non-absorbent material and covered with an absorbent layer such as a wrapping of cotton tape. Plugs 23 and 24 are used to form the inside ends of the piece to size. While these plugs are usually of the same composition as the mould 12 they may be of non-absorbent material in many cases. Where they are made of absorbent material, the inner ends are covered with non-absorbent material 25. In the casting operation the two halves of the mould are bolted together being made to register by dowels 26 which register with holes in the complementary half of the mould case. After the pipes 15 and 16 with the end plugs 23 and 24 are in place, the two halves may be clamped together through bolts placed in the holes 11. The plugs and pipe are held in proper position by collars 28 or other suitable means. In general the mould is then stood in a vertical position and casting slip admitted by opening the valves 17 and 18. When the mould is filled, preferably from the bottom, and slip begins to flow out of the pipe 19 the valve 17 may be closed. Pressure may then be placed on the slip inside the mould through the pipe 20 which causes the material to deposit much more rapidly than where the capillary attraction only is used to take out the water and build up the layer of material 14. The jacket 10 permits the use of rather high pressures. With the high pressure it is possible to maintain contact between the piece 14 and the surface of the mould 12 at all times. This permits the use of slip which otherwise would tend to contract and draw away and also makes it possible to build up a dense layer which will have less shrinkage in the drying operation. In some slips it is not necessary that pressure be applied in order to make use of the invention. In general, however, it is found advisable as the time of casting is materially reduced and a mould may be generally used which has much longer life.

When the cast piece has obtained the desired thickness which is usually determined by time or by noting the increase in the weight of the mould with slip as a whole, the pipe 19 is connected to an air or oil supply which has a pressure equal to, if not slightly greater, than that in the line 20. The valve 17 may then be opened allowing air or oil to enter which will replace the slip on the inside of the piece. In some cases it is desirable to disconnect the line 20, opening the valve 18 and drawing the slip 29 out of the interior of the piece, after which air or oil may be allowed to take its place.

The inner layer of the piece which has been in contact with the slip has a much larger percentage of water. When, however, the in-

terior of the piece is filled with air or oil under pressure, the water is driven out through the outer layer and the percentage of water between the inner and outer layers more nearly equalized. This tends to reduce the shrinkage on the inner surface and makes it possible to form pieces not otherwise possible. In some cases it is not possible to use air as it may tend to break through the piece. In most of these instances, however, oil, kerosene, or gasoline may be used to advantage. In general, it is advisable to use a material which will not wet or dissolve the inner surface as water would, but one which will tend to drive out the water and harden the inner surface. When the water on the inner surface has been reduced sufficiently, the pressure may be reduced and the oil removed from the inner surface. In some cases, it may be desirable to circulate air through the inner surface in order that the piece may be given a slight shrinkage, permitting it to be drawn more readily from the moulds. In many pieces, however, this method permits of making a piece sufficiently hard so that it may be readily removed from the moulds. In very delicate pieces it is frequently possible to fill the interior either partially or wholly with wax in place of oil or air. As the wax hardens it will form a support for the piece permitting it to be removed from the mould. Where the piece is placed in a warm room with a high degree of moisture saturation, the wax may be softened and permit contraction of the formed piece without damaging the piece.

The method may be applied in many different ways. It is important, however, to apply pressure to the inner surface after the forming in order to drive out excess water.

With the arrangement shown in the drawing, slip may be allowed to flow through the piece by regulating the valves 17 and 18. This tends to prevent settling of the slip which is especially important in casting electrical porcelain as resulting dielectric properties of the mixture may be spoiled by the settling operation. The circulation of the slip on the inside also tends to cause a more uniform composition on the walls of the piece. Where the absorbing material of the mould 12 is of a dense composition the absorption may readily be improved by the use of ducts 30 and 31 opening through perforations 32 in the outer case.

While the drawing shows a construction particularly adaptable for very high pressures, many pieces may be formed, particularly those of small size, by simply clamping the halves of the plaster moulds together with a clamp.

In the improved method it is possible to use a cement which has an open structure and which will not readily be dissolved by the water and salts absorbed from the casting

slip. The increased pressure possible permits of the use of moulds of greater density than would otherwise be possible. In some cases, the moulds themselves may be made of porous, vitreous material which has been fired. Where moulds of this kind are used, it is usually necessary to back them up with plaster or cement to take care of any irregularities. The surface tension of the liquid placed 10 on the inside of the piece after casting as well as the surface tension in the water in the built up material are important factors in eliminating the excess water on the inner surface and makes it possible to form pieces 15 which would otherwise crack in drying or burning or which could not be readily removed from the moulds.

It is evident that by starting the pressure rather low and increasing it that a more 20 uniform density of material will be obtained from the cast piece. It is, however, important that the expansion or deformation of the mould for different pressures be given careful consideration. In some cases it is desirable to start at a much higher pressure and 25 reduce the pressure as the operation proceeds. This is particularly true where the operation requires considerable time so that there is a slight shrinkage in the piece. By removing 30 the pressure as the operation proceeds, the mould will contract and take up the shrinkage so that the pressure on the inside of the piece will not cause a tension on the outer layer with the danger of forming a flaw.

35 In order to facilitate the draining or filling of the mould or cast piece of ware valves 34 and 35 may be added. The lines to which these valves are connected may be connected to an air or oil supply as desired.

40 I claim—

1. The method of casting comprising the steps of filling a mould of porous material with a ceramic ware slip, placing hydraulic pressure on the slip within the mould to facilitate passage of water from said slip to said mould, permitting a layer of ceramic material to be deposited on the inner wall of said mould, removing the slip from the mould, and filling the interior of the mould 45 with a fluid under pressure to compress the deposited layer and render it more nearly uniform.

50 2. The method of casting ceramic ware comprising the steps of filling a ceramic slip into a porous mould, permitting a deposit of ceramic material from said slip on the inner surface of said mould, draining the slip from the mould, filling the mould with a liquid immiscible with water and subjecting said liquid to pressure to compress said layer against the wall of said mould to render said layer more uniform.

55 3. The method of casting ceramic ware comprising the steps of filling slip into a porous mould and agitating the slip during

deposit of a layer therefrom on the surface of said mould.

4. The method of casting ceramic ware comprising the steps of filling a porous mould with slip, placing pressure on said slip to 70 facilitate the deposit of a layer therefrom on the surface of the mould and agitating the slip during the deposit of the layer.

5. The method of casting ceramic ware comprising the circulation of slip through a 75 porous mould to permit deposit of a layer therefrom on the surface of said mould.

6. The method of casting ceramic ware comprising the circulation of slip under pressure through a porous mould to permit deposit of a layer of material from said slip on the surface of the mold. 80

7. The method of casting ceramic ware comprising circulating slip through a ceramic mould to permit the deposit of a layer therefrom on the surface of the mould, removing the slip leaving the deposited layer and exerting pressure on said layer while still in said mould to remove moisture therefrom and render the layer more nearly uniform. 90

8. The method of casting ceramic ware comprising the steps of introducing slip into a lower part of the mould permitting the slip to escape from the upper part thereof and thereby causing the slip to circulate upward- 95

9. The method of casting ceramic ware comprising the steps of causing slip to enter at a porous bottom and to escape at the top of the mould, and providing resistance to 100 the escape of the slip to produce pressure on the slip in the mould.

10. The method of casting ceramic ware comprising the steps of introducing slip under pressure into a porous mould, permitting the slip to escape from the mould and offering resistance to escape of the slip from the mould to place the slip in the mould under pressure, thus supplementing capillary action in withdrawing liquid from the slip through 110 the walls of the mould. 105

11. The method of casting ceramic ware comprising the steps of placing slip under pressure in a porous mould, agitating the slip during deposit of material therefrom on the 115 inner surface of the mould and forcing the slip from the mould by means of fluid under a pressure sufficient to force the slip from the mould against the pressure thereon.

12. The method of casting ceramic ware comprising the introduction of slip into the lower portion of the mould, exerting pressure on the slip when the mould is filled therewith, permitting deposit of material from said slip on the wall of the mould and introducing a 120 liquid under pressure immiscible with the liquid of said slip into the upper portion of the mould, the pressure on said liquid being sufficient to force the slip from the mould against the pressure on the slip. 125

13. The method of casting ceramic ware comprising the deposit of a layer of material on the inner face of a porous mould from slip contained in the mould, removing the slip and introducing material to form a core on the interior of the formed layer.

14. The method of casting ceramic ware comprising the deposit of a layer on the inner surface of a mould from slip contained in the mould, and providing a yielding core within the interior of the formed layer.

15. The method of casting ceramic ware comprising the deposit of a layer on the inner surface of a porous mould from slip contained in the mould, and introducing solidifying material into said mould to form a core therein.

16. The method of casting ceramic ware

comprising the deposit of a layer on the surface of a porous mould, from slip held in the mould, withdrawing the slip and introducing material which solidifies into a yielding mass to form a core and exerting pressure on said layer by means of said material.

17. The method of casting comprising the steps of depositing a layer on the inner surface of a porous mould, from slip held in said mould, withdrawing the slip and introducing liquefied wax into the mould to exert pressure on the formed layer and maintaining the wax yielding during drying of said layer.

In testimony whereof I have signed my name to this specification on this 29th day of June A. D. 1926.

ARTHUR O. AUSTIN.